

## UNITED STATES PATENT OFFICE

2,162,938

GRANULAR ALUMINUM AND METHOD OF  
MAKING THE SAME

George F. Comstock and Viatcheslav V. Efimoff,  
Niagara Falls, N. Y., assignors to The Titanium  
Alloy Manufacturing Company, New York,  
N. Y., a corporation of Maine

No Drawing. Application April 10, 1936,  
Serial No. 73,640

25 Claims. (Cl. 75—27)

Our invention relates to the production of an improved granular aluminum that may be advantageously used in metallurgical reactions, more particularly as a reducing agent.

5 Metallurgical reactions performed by means of the well-known aluminothermic process require metallic aluminum in a finely divided form for mixing with the oxide of the other metal to be reduced. Aluminum powder such as is used for 10 paint pigment is not generally used for metallurgical reactions on account of its high cost, and aluminum shot formed by pouring molten aluminum into water is not satisfactory on account of its coarse size and compactness of form, 15 thereby giving slow and incomplete reactions.

The preferable form of aluminum for these reactions is known as "grained aluminum", and is produced by breaking up the metal mechanically just as it is passing from the liquid to the solid 20 state. Particles formed in this way are rough and cracked, if the breaking up has been accomplished at just the right temperature, and if they are also not too coarse, they react vigorously with metallic oxides.

25 We have now discovered that a new and improved form of grained aluminum may be readily produced by adding certain salts and compounds to the solidifying aluminum while it is being stirred vigorously.

30 We have also discovered that the vigor of the aluminothermic reaction in which this product is used may be controlled in a convenient way by adjusting the amount and kind of the compounds which are mixed with the aluminum while grain- 35 ing it.

Although these discoveries have been made by us after experimentation and tests, and are now utilized by us in the manufacture of ferrotitanium by the aluminothermic process, they are of 40 course applicable to grained aluminum in general, and for whatever metallurgical reactions that product may be applied to, such as the manufacture of nickel-titanium, ferro-chromium, ferro-zirconium, ferrocolumbium, ferro-molybdenum, etc., or in the direct manufacture 45 of alloy steel by the reduction of the oxide of the alloying element such as chromium, zirconium, titanium, columbium, etc., by means of our improved grained aluminum in the steel-melting furnace.

As one example of the application of our improved methods for making and using the improved form of grained aluminum, which is the 50 subject of our invention, the particular kind in-

tended for the manufacture of ferrotitanium will now be described.

Example A.—Aluminum of ordinary commercial purity was first melted at 1400° F. or higher in an oil-fired tilting crucible furnace, and at 5 convenient intervals 40 pounds were poured out and transferred to an iron pot over which a suitable stirring device was mounted. Our preferred type of stirring device consisted of a vertical shaft with a curved plate on the bottom end, the 10 curve being fitted approximately to the contour of the pot, and having a deeply toothed edge. The shaft was capable of being rotated, and also capable of being raised or lowered relatively to the pot. 15

After the molten aluminum was poured into the pot, the stirrer was placed in operation to agitate the molten aluminum while cooling, and a mixture consisting of 7 pounds of powdered synthetic cryolite (a mixture of sodium fluoride 20 and aluminum fluoride) and 7 pounds of powdered rutile (containing about 81%  $TiO_2$ , 3%  $SiO_2$  and balance  $Fe_2O_3$ ) was added to the pot.

The cryolite we used contained approxi- 25

|             | Per cent |
|-------------|----------|
| $Al_2F_6$   | 43.12    |
| NaF         | 55.90    |
| $Na_2SiF_6$ | 0.42     |
| $H_2O$      | 0.35 30  |
|             | 99.79    |

When these powders were thoroughly mixed with the partly frozen aluminum and the entire batch had cooled to a very dull red heat, around 35 1200° F., it was charged a little at a time into a suitable swing-hammer mill which effectively completed the granulation.

After passing through this mill the aluminum 40 was solid, and the mixture was thrown on an inclined screen of  $\frac{1}{8}$  inch mesh, the oversize being returned to the pot for softening and breaking up with the next batch.

In this way all the aluminum was eventually 45 utilized, the only losses being by oxidation in melting, and in dust from the hammer mill. These usually averaged about 9%.

Various salts or metallic compounds (milled to about 100 mesh or finer), such as sodium chloride, potassium chloride, sodium carbonate, magnesium chloride, ammonium chloride, and mixtures of them, have been tried by us in place of cryolite in our improved methods, but cryolite has been found most satisfactory for the grain- 50 ing process. The graining process was also tried 55

without any salt addition, but it was extremely difficult and laborious to secure fine grains in that way, more than 50% oversize invariably being obtained.

- 5 As examples of the use of various salts to assist in the graining of aluminum by improved methods the following experiments may be mentioned. Fifteen pounds of aluminum were melted in the graining pot, and the dross was skimmed off.
- 10 The molten metal was stirred 9 minutes mechanically, while cooling, and during that time 4 pounds 7 ounces of powdered common salt (commercial sodium chloride) were added gradually. This salt had been powdered by milling for one 15 and one-half hours in an iron ball mill. After this addition, stirring by hand was continued until the lumps were too cold to be broken up. The product was then washed with hot water, and when thoroughly washed and dried, it was 20 screened through an 8 mesh screen. The aluminum remaining on the screen was 6 pounds 6 ounces while 8 pounds 7 ounces passed through. The production of fines was thus 56%.

When this method was repeated using 3.75 pounds of powdered cryolite (a mixture of 43% aluminum fluoride, 56% sodium fluoride, and 1% sodium silico-fluoride, moisture, etc.), instead of the sodium chloride, and without washing of the product, we obtained 16 pounds 6 ounces fines 30 through an 8 mesh screen, and only 1 pound 12 ounces of oversize, or a yield of 87.5% fines.

When repeated by using for the graining agent 5.25 pounds of a mixture consisting of 40% soda ash (commercial sodium carbonate), 22% commercial sodium chloride, and 38% commercial potassium chloride, the method yielded a product which, after thorough washing and drying, consisted of 10 pounds 14 ounces of granular aluminum finer than 8 mesh and 4 pounds 10 ounces 40 of coarser particles, thereby indicating a production of 72.5% fines.

Other mixtures of salts were also tried with much inferior results, and we therefore decided that cryolite was more satisfactory than other 45 salts having lower melting points.

The use of cryolite to assist the graining has the further advantage that its presence with the grained aluminum improves the reactivity of the latter when it is used as a reducing agent in 50 metallurgical work. Cryolite, in fact, has been found to be practically indispensable as a flux when aluminum is so used, and the advantage of having this flux intimately associated with the aluminum grains is therefore obvious. By our 55 improved methods the aluminum grains become coated with the cryolite flux instead of carrying a coating of refractory aluminum oxide which is unavoidably formed when the graining operation is attempted in air without the aid of any 60 salt such as cryolite.

The amount of cryolite used has been varied between zero and 27.4% of the total mixture. When less than about 10% was used, the graining operation was difficult (unless other 65 pounds such as rutile were used in addition); and when more than about 20% cryolite was added, the aluminothermic reactions in which the grained aluminum was used were too violent.

For example, in making ferrotitanium with 70 this improved grained aluminum, a reaction, in which 138 pounds of grained aluminum containing 24.5% of cryolite was used, lasted only 1½ minutes, and yielded 15 pounds of metal; while another one made with the same amount of the 75 same kind of mix, except that the grained alu-

minum contained only 13.5% of cryolite lasted nearly 2 minutes and yielded 66 pounds of metal.

Since the manufacture of grained aluminum was facilitated by the addition of over 20% of powdered nonmetallic compounds (such as 5 cryolite), while stirring the freezing metal, and the presence of so much cryolite in the grained aluminum made it too reactive for more effective use, the substitution of a less active ingredient for some of the cryolite was tried.

10 The most useful ingredient for this purpose would naturally be the oxide of the metal for the reduction of which the grained aluminum is to be used. Rutile, for instance, has been used when ferrotitanium was to be produced, and pure 15 titanium oxide when nickel titanium was the final objective.

Similarly other oxides may be used when other alloys are to be made. The amount of rutile or other metallic oxides which we have used has 20 ranged ordinarily from zero to about 17%, but for special purposes, such as the direct manufacture of alloy steel by the addition of grained aluminum and the oxide in a steel-melting furnace, any proportions up to two or more of oxide to one 25 of aluminum may be advantageously employed. The proportions noted in Example A, namely 13% each of cryolite and rutile, we have found to be very satisfactory for grained aluminum to be used in the manufacture of ferrotitanium by 30 the aluminothermic process; such graining operation is easy, and an average reaction using 130 pounds of the product and lasting about 2 minutes gives a yield of 85 to 100 pounds of high 35 quality alloy.

To make an aluminum-rutile mixture with approximately equal parts of each in a fine-grained form, 30 pound batches of molten aluminum were poured off into the graining pot, and to each one 5 pounds of cryolite and 25 pounds of 40 fine rutile were added while stirring. The analyses of these materials have been heretofore given in this example.

In order to obtain proper graining of the aluminum and also to avoid the formation of coarse 45 lumps from too rapid chilling, it was found necessary to preheat these large additions of rutile. This was most conveniently accomplished by placing the rutile and cryolite in the graining pot first, and heating them there to about 800° or 50 900° F. The molten aluminum was then poured on top, and after stirring vigorously while cooling, and also passing through the swing-hammer mill when cooled to a pasty condition, a well-grained mixture was obtained. From two batches 55 of the quantities mentioned, the yield was 101 pounds of product passing an 8 mesh screen, with 7 pounds oversize.

Two other batches were made using even more 60 rutile, or in the proportion of 40 pounds of preheated fine rutile, 3 pounds of cryolite, and 20 pounds of molten aluminum. This also gave a good granular mixture, 97 pounds from the two batches passing through the 8 mesh screen, with 11 pounds oversize, the balance being chiefly 65 dust loss because the rutile was rather fine.

It is thus evident that our improved graining methods are practical for the production of a mixture containing twice as much, or more, of a 70 reducible oxide as of the granular aluminum reducing agent, when such a mixture is desired for furnace additions.

Example B.—The following example illustrates the use of our new granular aluminum in the manufacture of nickel-titanium. Aluminum was 75

5 melted, transferred in 39 pound batches to the  
graining pot, stirred and passed through the  
swing-hammer mill as described in Example A,  
but the addition consisted only of 9 to 10 pounds  
10 of cryolite for each batch. This operation was  
repeated for 15 batches which yielded 86% of the  
original materials as an aluminum-cryolite mix-  
ture through an 8 mesh screen, the missing 14%  
15 being accounted for by dross formed in melting,  
dust losses, and oversize.

Then 41 pounds of this product mixed with  
black nickel oxide (containing over 99%  $\text{Ni}_2\text{O}_3$ ,  
and less than 1%  $\text{Fe}_2\text{O}_3$ ,  $\text{CuO}$ , and other impuri-  
ties), and of rutile containing 94.7%  $\text{TiO}_2$ , 2.16%  
15  $\text{Fe}_2\text{O}_3$ , 0.97%  $\text{SiO}_2$ , and 2.17%  $\text{CaO}$ ,  $\text{Al}_2\text{O}_3$ , and  
other impurities, was milled to a fine powder in  
a ball mill, then packed in a suitable container,  
and ignited.

20 After the reaction 35 pounds of alloy contain-  
ing 28.8% titanium, 7.64% aluminum, 2.8% iron,  
1.11% silicon and balance nickel (about 59.65%)  
were recovered, whereas by using commercial  
25 finely divided aluminum plus a proportional  
amount of cryolite in a similar mix and process,  
only 32.5 pounds of alloy containing 26.7%  
titanium were obtained.

Example C.—The following example shows the  
use of our improved methods in the manufacture  
30 of ferro-chromium. Grained aluminum was pre-  
pared exactly as described in Example A, except  
that in place of 7 pounds of fine rutile per batch  
of 40 pounds of aluminum, 7 pounds of fine-  
grained chrome ore were used. The cryolite was  
35 used in the same way as with rutile. The chrome  
ore contained approximately 47%  $\text{Cr}_2\text{O}_3$ , 21%  
 $\text{FeO}$ , 15%  $\text{MgO}$ , 11%  $\text{Al}_2\text{O}_3$ , 5%  $\text{SiO}_2$ , and 1%  
 $\text{CaO}$ . This gave just as good results as rutile in  
40 graining, and from 80 pounds of molten alu-  
minum, 14 pounds of cryolite and 14 pounds of  
chrome ore, 95 pounds of the grained mixture  
45 passing through an 8 mesh screen were recovered  
with 9.5 pounds oversize.

The fine product was used as a reducing agent  
for making ferro-chromium in the following way:  
45 A mixture consisting of 65 pounds of the low-  
grade chrome ore as before described, 25 pounds  
of the grained-aluminum with cryolite and  
chrome ore, 3 pounds of calcium silicide (con-  
50 taining about 30% calcium, 3% iron, and balance  
silicon), and 5 pounds of cryolite was milled in an  
iron ball mill for 15 hours, and then 3 pounds of  
magnesium shavings and 10 pounds of sodium  
55 chlorate were added, and then mixed for half  
an hour longer in the same mill. This mix was  
packed in a suitable container and ignited. A  
violent reaction occurred, and the alloy recovered  
weighed 21.5 pounds and contained 50.32% chro-  
60 mium, 35.73% iron, 8.54% silicon, and the bal-  
ance chiefly aluminum.

65 Example D.—The following example shows the  
use of our improved methods in the manufacture  
of ferro-aluminum-zirconium: Grained alu-  
minum was prepared exactly as described in  
Example A, except that in place of 7 pounds of  
fine rutile per batch of 40 pounds of aluminum, 7  
pounds of fine zirconium oxide was used. The  
cryolite was used in the same way as with rutile.  
The zirconia contained approximately 95%  $\text{ZrO}_2$ ,  
4%  $\text{SiO}_2$ , and 1% impurities, including  $\text{TiO}_2$ ,  
70  $\text{Fe}_2\text{O}_3$ ,  $\text{Al}_2\text{O}_3$ , etc. This gave nearly as good re-  
sults as rutile in graining, and from 80 pounds  
of molten aluminum, 14 pounds of cryolite and  
14 pounds of zirconia, 91 pounds of the grained  
75 mixture passing through an 8 mesh screen were  
recovered, with 7.5 pounds oversize.

The fine product was used as a reducing agent  
for making ferro-aluminum-zirconium in the fol-  
lowing manner. A mixture consisting of 25  
pounds of zirconia as hereinbefore described, 35  
pounds of the grained aluminum with cryolite and zir-  
5 conia, 10 pounds of sodium chlorate, and 10  
pounds of cryolite was mixed in an iron ball mill  
for half an hour, then packed in a suitable con-  
tainer and ignited. A violent reaction occurred,  
10 and the alloy recovered weighed 22 pounds and  
contained 13.57% zirconium, 64.62% iron, 2.14%  
silicon and 19.67% aluminum.

The same kinds of grained aluminum could,  
of course, be equally well applied to the manu-  
facture of ferro-zirconium or ferro-chromium, re-  
spectively, of different grades than those men-  
tioned in these Examples C and D by varying the  
proportions of the oxides and reducing agent  
used.

20 In applying this improved grained aluminum  
to the reduction of alloying elements directly  
from their oxides into a bath of steel or other  
metal in a melting furnace, it might be advisable  
25 under certain conditions to have the material  
coarser than the 8 mesh and finer size which has  
been used successfully for alumino-thermic re-  
actions in cold crucibles. The grained aluminum  
product containing mixed cryolite or other salt,  
30 and with or without a metallic oxide or several  
such oxides in addition, might even be briquetted  
to advantage for such a use, so as to form larger  
compact masses for easy charging through a  
furnace door onto a molten metal bath.

Our invention is therefore not confined to a  
35 fine-grained product, but is also applicable to  
grained aluminum of any size or in briquetted  
form.

If for some special purpose a pure grained  
aluminum is desired, our improved methods of  
40 graining may be carried out advantageously with  
a water-soluble salt, such as sodium chloride in  
a fine grained form. By a simple leaching in  
water after the mixture of grained aluminum and  
salt has passed through the hammer mill, the salt  
45 is removed, and the aluminum granules are left  
in a pure state.

We claim as our invention:

1. A granular metallurgical reducing agent  
45 consisting of finely-divided aluminum particles  
coated with cryolite.

2. In the method of making grained aluminum  
from molten aluminum, the step which consists  
50 in adding to the molten metal while freezing and  
with stirring powdered cryolite to produce granu-  
lation.

3. In the method of making a granular metal-  
lurgical reducing agent from molten aluminum,  
the step which consists in adding to the molten  
55 metal while freezing and with stirring powdered  
cryolite and rutile to produce said granular re-  
ducing agent.

4. In the method of making a granular metal-  
lurgical reducing agent from molten aluminum,  
the step which consists in adding to the molten  
65 metal while freezing and with stirring powdered  
cryolite and an oxide of a reducible metal to  
produce said granular reducing agent.

5. In the method of making a ferrotitanium  
70 alloy by the aluminothermic process, the step  
which consists in mixing as a reducing agent  
with the titanium ore granular aluminum inti-  
mately mixed with and having adhered thereto  
particles of powdered cryolite.

6. In the method of making a ferrotitanium 75

alloy by the aluminothermic process, the step which consists in mixing as a reducing agent with the titanium ore granular aluminum intimately mixed with and having adhered thereto particles of powdered cryolite and rutile.

7. In the method of making a nickel-titanium alloy by the aluminothermic process, the step which consists in mixing as a reducing agent with nickel and titanium oxides granular aluminum intimately mixed with and having adhered thereto particles of powdered cryolite.

8. In the method of making alloy steels, the step which consists in adding to the molten steel granular aluminum intimately mixed with and having adhered thereto particles of powdered cryolite and a powdered oxide of the alloying element to be reduced into the steel.

9. A granular metallurgical reducing agent consisting of finely-divided aluminum particles intimately mixed with and having adhered thereto particles of powdered cryolite.

10. A granular metallurgical reducing agent consisting of finely-divided aluminum particles intimately mixed with and having adhered thereto particles of powdered cryolite and powdered rutile.

11. A granular metallurgical reducing agent consisting of finely-divided aluminum particles intimately mixed with and having adhered thereto particles of equal amounts of powdered cryolite and powdered rutile.

12. A granular metallurgical reducing agent consisting of finely-divided aluminum particles intimately mixed with and having adhered thereto particles of powdered cryolite and a powdered oxide of a reducible metal.

13. A granular metallurgical reducing agent consisting of finely-divided aluminum particles intimately mixed with and having adhered thereto particles of equal amounts of powdered cryolite and a powdered oxide of a reducible metal.

14. A granular metallurgical reducing agent for aluminothermic reactions composed of finely-divided aluminum intimately mixed with and having adhered thereto particles of one or more powdered salts selected from the group consisting of cryolite, sodium chloride, potassium chloride, sodium carbonate, magnesium chloride and ammonium chloride.

15. A granular metallurgical reducing agent for aluminothermic reactions composed of finely-divided aluminum intimately mixed with and having adhered thereto particles of one or more powdered salts selected from the group consisting of cryolite, sodium chloride, potassium chloride, sodium carbonate, magnesium chloride and ammonium chloride in an amount ranging from 5% to 200% of the aluminum present.

16. A granular metallurgical reducing agent for aluminothermic reactions composed of finely-divided aluminum intimately mixed with and having adhered thereto particles of one or more powdered salts selected from the group consisting of cryolite, sodium chloride, potassium chloride, sodium carbonate, magnesium chloride and ammonium chloride and also with a powdered oxide of a reducible metal.

17. A granular metallurgical reducing agent for aluminothermic reactions composed of finely-divided aluminum intimately mixed with and having adhered thereto particles of one or more powdered salts selected from the group consisting of cryolite, sodium chloride, potassium chlo-

ride, sodium carbonate, magnesium chloride and ammonium chloride in an amount ranging from 5% to 200% of the aluminum present and also with a powdered oxide of a reducible metal.

18. A granular metallurgical reducing agent for aluminothermic reactions composed of finely-divided aluminum intimately mixed with and having adhered thereto particles of powdered cryolite in an amount ranging from 5% to 35% of the mixture.

19. A granular metallurgical reducing agent for aluminothermic reactions composed of finely-divided aluminum intimately mixed with and having adhered thereto particles of powdered cryolite in an amount ranging from 2% to 25% of the mixture, and also with a powdered oxide of a reducible metal in an amount ranging from 2% to 70%.

20. A granular metallurgical reducing agent for aluminothermic reactions composed of aluminum mixed while molten with one or more powdered salts selected from the group consisting of cryolite, sodium chloride, potassium chloride, sodium carbonate, magnesium chloride and ammonium chloride, and granulated while mixed with the solid salts whereby the particles of aluminum and salts adhere to one another.

21. In the method of making grained aluminum from molten aluminum, the step which consists in adding to the molten metal, while freezing and with stirring, one or more powdered salts selected from the group consisting of cryolite, sodium chloride, potassium chloride, sodium carbonate, magnesium chloride and ammonium chloride to produce granulation.

22. In the method of making grained aluminum from molten aluminum, the step which consists in adding to the molten metal, while freezing and with stirring, one or more powdered salts selected from the group consisting of cryolite, sodium chloride, potassium chloride, sodium carbonate, magnesium chloride and ammonium chloride, and a powdered oxide of a reducible metal to produce granulation.

23. In a method of making grained aluminum from molten aluminum, the step which consists in adding to the molten metal, while freezing and with stirring, one or more powdered salts selected from the group consisting of cryolite, sodium chloride, potassium chloride, sodium carbonate, magnesium chloride and ammonium chloride at temperatures lower than that of the freezing molten metal to produce granulation.

24. In the method of producing metallurgical reactions to form alloys by the aluminothermic process, the step which consists in mixing as a reducing agent with the oxide of the alloying element finely-divided aluminum intimately mixed with and having adhered thereto particles of one or more powdered salts selected from the group consisting of cryolite, sodium chloride, potassium chloride, sodium carbonate, magnesium chloride and ammonium chloride.

25. In the method of producing metallurgical reactions to form alloys by the aluminothermic process, the step which consists in mixing as a reducing agent with the oxide of the alloying element finely-divided aluminum intimately mixed with and having adhered thereto particles of powdered cryolite.